

Oct. 28, 1958

N. J. KODA ET AL

2,858,463

STORAGE SCREEN FOR DIRECT-VIEWING STORAGE TUBE

Filed July 1, 1955

2 Sheets-Sheet 1



FIG. 1.



FIG. 2.



FIG. 3.



INVENTORS.  
SIDNEY T. SMITH,  
NOBUO J. KODA,  
BY  
Henry Heyman  
ATTORNEY.

Oct. 28, 1958

N. J. KODA ET AL

2,858,463

STORAGE SCREEN FOR DIRECT-VIEWING STORAGE TUBE

Filed July 1, 1955

2 Sheets-Sheet 2



FIG. 5.



FIG. 6.

FIG. 7.



FIG. 8.



FIG. 9.



FIG. 10.

INVENTORS.  
SIDNEY T. SMITH,  
NOBUO J. KODA,  
BY

Henry Heyman

ATTORNEY.

1

2,858,463

## STORAGE SCREEN FOR DIRECT-VIEWING STORAGE TUBE

Nobuo J. Koda, Culver City, and Sidney T. Smith, Pacific Palisades, Calif., assignors to Hughes Aircraft Company, Culver City, Calif., a corporation of Delaware

Application July 1, 1955, Serial No. 519,384

3 Claims. (Cl. 313—68)

This invention relates to direct-viewing storage tubes and more particularly to a process for making an improved storage screen for use therein that has uniform control and cut-off characteristics providing an extended cut-off range.

The present invention is directed towards the fabrication of an improved storage screen for use in the direct-viewing half-tone storage device disclosed in a copending application, now Patent No. 2,790,929 entitled "Direct-Viewing Half-Tone Storage Device," issued to E. E. Herman and G. F. Smith on April 30, 1957, and assigned to the same assignee as the present invention. In the Smith et al. patent, a direct-viewing half-tone storage device is disclosed which incorporates a storage screen comprising an electroformed nickel screen having patches of dielectric material of uniform thickness distributed uniformly over approximately 50% of the exposed surface on one side of the meshes thereof. In the operation of a tube of this type, a charge pattern is produced on the storage screen which, in turn, controls the flow of flood electrons to a viewing screen to produce a visual presentation of the charge pattern.

It is highly desirable that individual interstices or holes in the storage screen have uniform control over the flow of flood electrons over the entire storage screen. The advantage of this is that a storage element of information on the storage screen can be of the same order of magnitude as an individual hole. On the other hand, if individual holes in the storage screen have random control with an average near the desired value, a storage element of information on the storage screen must contain approximately at least 10 individual holes or control elements to provide a true representation of the desired average control. Also, in conjunction with the above, it is desirable that the individual interstices of storage screen have a uniform extended cut-off characteristic. As disclosed in the Herman et al. patent, an extended cut-off characteristic was achieved by covering only a portion of the meshes of the screen with dielectric material. This extended cut-off characteristic, however, was not uniform for each interstice of the storage screen as is the storage screen of the present case.

In accordance with the present invention, a process is disclosed for fabricating a storage screen wherein the dielectric material is disposed symmetrically about each interstice which may be circular or square. When this condition exists, each interstice of the screen exerts the same control over the flow of flood electrons. In the preferred embodiment of this screen, a thin layer of dielectric material is disposed on the central portion of each mesh of an electroformed screen. An advantage of having the layer of dielectric material disposed on the meshes of the conductive screen in this manner is that the erasure speed is increased, i. e., the storage surface can be charged in a negative direction more efficiently. To erase stored images or to provide a negative background for good contrast the dielectric material is charged

2

negatively with low velocity electrons having a secondary emission ratio less than unity. The electric field from the viewing screen penetrates the interstices of the storage screen and influences the electric field immediately adjacent the layer of dielectric storage material. This is particularly true for highly transparent, coarse storage screens. During the erasure process this field from the viewing screen causes some of the low-velocity flood electrons to be deflected away from the storage surface, to fall into the interstices, and to ultimately strike the viewing screen. This action results in a loss of erasure electrons and contributes to the objectional bright flash on the viewing screen during erasure. In the case of the present invention the layer of dielectric material, due to its central location, is shielded by a maximum amount from the influence of the viewing screen field. This would eliminate the need for lowering the potential applied to the viewing screen during erasing intervals.

The process for fabricating a storage screen of this type comprises first evaporating a dielectric material over one side of an electroformed screen without depositing any dielectric material within the interstices thereof. This may be accomplished, for example, by the use of a material known as photo resist in a manner hereinafter explained. After the dielectric material has been evaporated on the screen, the meshes of the screen are then increased to the desired width by plating additional metal on the exposed conductive portions of the surfaces thereof.

It is therefore an object of the invention to provide a process for fabricating an improved storage screen adaptable for use in a direct-viewing storage device.

Another object of the invention is to provide a storage screen capable of being more efficiently erased and having uniform control characteristics in each interstice of its entire area.

Still another object of the present invention is to provide a process for fabricating a storage screen having a thin layer of dielectric material disposed symmetrically over only a portion of the exposed surface on one side of the meshes of an electroformed screen.

The novel features which are believed to be characteristic of the invention, both as to its organization and method of operation, together with further objects and advantages thereof, will be better understood from the following description considered in connection with the accompanying drawings in which an embodiment of the invention is illustrated by way of example. It is to be expressly understood, however, that the drawings are for the purpose of illustration and description only, and are not intended as a definition of the limits of the invention.

Figs. 1 and 2 are plan and cross-sectional views, respectively, of an enlarged portion of the storage screen of the present invention;

Figs. 3 and 4 are plan and cross-sectional views, respectively, of an enlarged portion of an electroformed screen; and Figs. 5 to 10 illustrate steps in the process of fabricating the storage screen shown in Figs. 1 and 2.

Referring now to the drawings, Figs. 1 and 2 show plan and cross-sectional views, respectively, of an embodiment of the storage screen of the present invention. More particularly, the storage screen comprises a metallic screen 10 having of the order of 250 meshes per inch, a thickness of 0.001 inch, and a transparency of approximately 40%. Along the central portion of the meshes of screen 10 is disposed a layer 12 of dielectric material such as, for example, magnesium fluoride. Thus, layer 12 has the configuration of a "dielectric screen" that is disposed in register with the metallic screen 10. The width of the meshes forming the dielectric screen, however, is approximately only one-half the width of the meshes of screen 10. The thickness of the layer 12 of

dielectric material is not critical and may, for example, be from 1 to 10 microns thick.

In accordance with the present invention, the storage screen described above is fabricated by commencing with an electroformed nickel screen 14 (Fig. 2) having the requisite number of meshes per inch and a thickness of the order of 0.0006 inch. The width of the meshes of screen 14, however, is made to be substantially equal to that of the dielectric screen formed by the layer 12. A plan and a cross-sectional view of an enlarged portion of the nickel screen 14 are shown in Figs. 3 and 4, respectively. The nickel screen 14 is stretched taut in a jig 16 as shown in Fig. 6.

The first principal step in fabricating the storage screen of the present invention, is to dispose the layer 12 of dielectric material on one side of the meshes of the nickel screen 14 without depositing any dielectric material on the inner surface of the interstices thereof. Conventional evaporation techniques have been found to be unsatisfactory as some molecules of the dielectric material are deposited within the interstices of the nickel screen 14 which result in non-uniformities in the finished storage screen. This step, however, may be accomplished by first coating the entire surface of the nickel screen 14, as shown in Fig. 5, with a layer 18 of photo resist in the absence of light. Photo resist may comprise, for example, a photosensitive lacquer or gelatin that is characterized by the fact that it is hardened by exposure to light. Prior to this, it may be dissolved in a liquid such as water or alcohol, depending on the type of photo resist employed. Also, the photo resist that is hardened by exposure to light may be removed by raising it to an appropriate temperature determined by its composition or by dissolving it in an appropriate chemical solution.

The portions of the layer 18 of photo resist on one side of the nickel screen 14 and on the inner surface of the interstices thereof are exposed to light thereby hardening these portions. This exposure may be made by projecting light towards one side of the coated screen 14 at a slight angle with the normal thereto in the manner shown in Fig. 6. To accomplish this, several sources of light may be employed or alternatively, the jig 16 in which the coated screen 14 is mounted may be rotated while being exposed so that light will be projected over the entire inner periphery of each interstice of the coated screen 14. The portions of the layer 18 of photo resist exposed to the light will be hardened. These portions are indicated by the shaded areas 20 of Fig. 7. The unexposed portions of layer 18 are indicated by the dotted areas 22 in the same figure.

After exposure to the light, the layer 18 of photo resist is then developed, i. e., the coated screen 14 is immersed in a liquid capable of dissolving the unhardened portions. Thus, the dotted areas 22 of layer 18 are washed away leaving only the hardened portions 20 as shown in Fig. 8. After this step of the process, only one side of the meshes of the nickel screen 14 remains uncoated. The thin layer 12 of dielectric material such as, for example, magnesium fluoride, may now be evaporated on the uncoated side of the meshes of the nickel screen 14. When magnesium fluoride is used, it is desirable to heat the screen 14 to a temperature of the order of 150° to 300° C. in order to get a good bond between the magnesium fluoride and the nickel. In that the photo resist layer 18 has a finite thickness, some dielectric material will be deposited on the exposed areas of the remaining hardened portions 20 as shown in Fig. 9.

After evaporation of the layer 12 of dielectric material, the nickel screen 14 is placed in an appropriate medium

and heated to a temperature necessary to "burn" the hardened portion 20 of the photo resist layer 18 off of the screen 14 or in an appropriate chemical solution to dissolve the hardened photo resist away. The actual composition of the medium or chemical solution and the necessary temperature will depend on the type of photo resist employed in the process. As mentioned above, a portion of the layer 12 of dielectric material will have been disposed on top of the hardened portion 20 of photo resist layer 18 which has now been burned away. This portion of the layer 12 will thus be left unsupported. Thence, in view of the fact that the layer 12 of dielectric material is only from 1 to 10 microns thick, the unsupported portions thereof may be broken away by agitating the screen 14 in water or other liquid, or by blowing air over and through the screen 14. After this step has been completed, the nickel screen 14 has the layer 12 of dielectric material disposed on only one side of the meshes thereof as shown in Fig. 10.

20 A coating 24 of metal (see Figs. 1 and 2) is now electroplated on the nickel screen 14 to increase the area of conductive surface surrounding the dielectric. The extent or amount of this plating generally represents a compromise between the percentage of conductive surface desired relative to the area of the layer 12 of dielectric material and the ultimate transparency of the storage screen. In the event that it is desired to plate copper on the exposed portions of nickel screen 14, the nickel screen 14 supported by the jig 16 is immersed in a saturated solution of electrolyte such as, for example, copper sulfate with the layer 12 facing and parallel to an anode. A small direct-current voltage of the order of 1 volt is developed between the anode and the nickel screen 14. For a screen of the order of 5 inches in diameter, one volt will cause a current of the order of 3 amperes to flow. During the plating operation, the nickel screen 14 is periodically rinsed with water and rotated in the plane parallel to the anode. The electrolyte may also be agitated or stirred to improve the uniformity of the plating. 30 The plating operation is continued until the desired increase in the width of the meshes of the nickel screen 14 has been achieved.

What is claimed is:

1. In a direct-viewing storage device, a storage screen comprising a conductive screen, and a continuous layer of dielectric material disposed about and spaced substantially uniformly from the periphery of each interstice of said screen on one side of the meshes thereof.

2. In a direct-viewing storage device, a storage screen comprising an electroformed metallic screen, and a continuous layer of dielectric material having secondary electron emission characteristics disposed about and substantially uniformly spaced from the periphery of each interstice of said screen on one side of the meshes thereof, the thickness of said layer being small relative to the thickness of said screen.

3. In a direct-viewing storage device, the storage screen as defined in claim 2 wherein the area of said continuous layer of dielectric material is substantially equal to the portion of the area of said meshes remaining exposed on said one side.

#### References Cited in the file of this patent

#### UNITED STATES PATENTS

|    |           |                       |               |
|----|-----------|-----------------------|---------------|
| 65 | 2,156,435 | Schroter et al. ----- | May 2, 1939   |
|    | 2,287,415 | Bwinett -----         | June 23, 1942 |
|    | 2,539,422 | Larson -----          | Jan. 30, 1951 |
|    | 2,682,501 | Teal -----            | June 29, 1954 |
| 70 | 2,685,660 | Norgaard -----        | Aug. 3, 1954  |
|    | 2,754,449 | Farnsworth -----      | July 10, 1956 |